

Feb. 1, 1944.

J. T. SCULLY ET AL

2,340,493

METHOD OF CASTING METAL INGOTS AND APPARATUS THEREFOR

Filed May 4, 1942

FIG. 1



Patented Feb. 1, 1944

2,340,493

# UNITED STATES PATENT OFFICE

2,340,493

## METHOD OF CASTING METAL INGOTS AND APPARATUS THEREFOR

John T. Scully, Lawrence, N. Y., and George H. Wyckoff, Mountain Lakes, N. J.

Application May 4, 1942, Serial No. 441,682

27 Claims. (Cl. 22—67)

The present invention relates to the art of casting ingots and has especial reference to a method and apparatus for casting ingots of steel or alloys of steel for later rolling or other mechanical working.

Among the general objects of the invention is the provision of a method of casting ingots whereby the ingot is formed with a thick side skin; the provision of a method of casting an ingot which will have a thick skin of substantially uniform thickness for a major portion of its length; the provision of a method for providing an ingot with a relatively deep zone, radially, of fine grain to present a strong surface or near surface zone for mechanical working, for example such as rolling; to reduce cavities, blow holes and the like; and to generally improve the soundness of ingots.

A further object is the provision of an improved method of casting ingots which are to be charged hot into soaking pits or reheating furnaces, for bringing the ingots to uniform and proper rolling temperature, which will provide a zone of fine grain for considerable radial depth by virtue of side wall cooling by the mold and which will provide compensation, or partial compensation, for the loss of ingot heat by side wall cooling by supplying, while the ingots are in the molds, heat at relatively high temperature, or temperatures, as the case may be, to the lower portion of the mold, heat which is of relatively high temperature to and below the solidification temperature of the grade of steel or alloy of steel cast, and in suitable volume, and thereby reduce the length of time required for such ingots to remain in the soaking pit or reheating furnace to reach the uniform and proper temperature preparatory to rolling.

A still further object is the provision of an improved method whereby ingots which are to be charged hot into a soaking pit or reheating furnace will be provided with a thick skin of fine grain for considerable inward or radial depth of substantially uniform thickness for the major portion of their lengths and in which heat loss to the bottom of the mold from the ingot will be considerably retarded by supplying external generated heat at relatively high temperature and suitable volume to the lower portion of the mold, and thereby reduce the length of time required for such ingots to remain in the soaking pit or reheating furnace to reach the uniform and proper temperature preparatory to rolling.

A still further object is the provision of a method whereby ingots which have been provided with

a thick skin by prolonged conductivity of heat in side wall cooling will be spaced from the inner side wall of the mold at or near stripping time and thereby facilitate complete stripping by the

5 crane.

A still further object is the provision of a method of casting ingots in big-end-down molds having ingot-forming chambers of tapering cross-section in which the vertical mold body is forced 10 against the skin or shell while the interior is molten and causes the molten interior to be squeezed upwardly.

15 A further important object is the provision of a method whereby ingots cast in big-end-down molds having ingot-forming chambers of tapering cross-section will be side wall cooled in the early stage of the casting substantially uniformly inwardly and the normal length of time of contact between the ingot skin and mold wall 20 will be increased by a relative body movement therebetween, and in the later stage will be cooled progressively upwardly.

25 Further objects are the provision of apparatus, in which the method may be carried out, which is simply constructed, inexpensive, durable, easily assembled and manipulated; which will provide efficient control of the operation; and which will facilitate stripping of ingots with a minimum risk of damage to their skins.

30 Other objects will hereinafter appear.

During casting of steel ingots the side surfaces of the poured molten mass are cooled relatively quickly by the side walls of the mold and a skin is formed which gradually grows in thickness as 35 more and more heat is absorbed by the side walls of the mold and which in cooling tends to shrink away from the side walls of the mold. As the process of solidification progresses the growing skin or shell builds up into thicker walls 40 rounding a diminishing molten interior and the thicker walls continue to grow toward the center. As the skin or outside of the ingot becomes solid metal and the hotter interior continues to cool and contract, the skin shrinks away from the side 45 walls of the mold and becomes spaced therefrom by an air gap, the loss of contact with the mold wall stops the direct conductivity of heat from the solidifying mass and the result is slower cooling and enlargement in crystal growth. Also, 50 by the manner of solidification combined with natural physical laws certain defects are produced in ingots such as segregation, top cavities, or pipe, or blowholes and pipe. The air gap formed between skin and mold side wall in big-end-down molds having tapering ingot-forming

chambers is relatively large due to the form of the molds and the direction of ingot shrinkage and settling relative to the direction of increased width of mold chamber, the gap being further enlarged or tending to further enlargement upon expansion of the mold. If the forming ingot and mold side walls are kept in contact for an increased length of time, other factors being the same, the skin or shell of the ingot becomes a thicker shell of small crystals resulting in a stronger and deeper zone for mechanical working thereon, for example, rolling, and if this deeper zone of fine grain is of uniform or substantially uniform thickness for the major portion of the length of the ingot it is a desirable advantage in subsequent mechanical working. Further, if in a big-end-down mold sufficient force be exerted on the mold body so that the tapering chamber wall will cause the skin or shell of the solidifying ingot to be moved laterally inwardly while the interior of the ingot is still molten, preferably for considerable depth, and is rigidly supported at its base, the result will be a squeeze upwardly of the molten interior which however slight will reduce the depth of top cavities or pipes, or in the case of molds equipped with hot tops will reduce the amount of molten metal required in the hot top to feed downwardly.

Steel ingots which are intended to be charged hot in soaking pits or reheating furnace to have their temperature equalized or brought to uniformity throughout preparatory to rolling are in common practice, considered by large producers as best practice, stripped from the molds as soon possible after pouring in order that they may be charged in the soaking pits before much of their original heat is lost thereby being brought to the uniform and proper rolling temperature quickly and also keeping low the fuel cost of the reheating furnace which at best is economically inefficient and expensive. The time at which it is practicable to strip ingots varies under well known conditions, it being customary for reasons above cited to strip a great percentage of ingots while their interiors are still molten and to allow many ingots, such as those of high carbon content and alloy steels to remain in their molds until their interiors have become completely solidified, and, as is well known, the solidification range of different steels varies widely, the difference being so much as 800°, or approximately as much, for high carbon steels containing more than 0.85 per cent carbon, the solidification temperature for these ranges in Fahrenheit from approximately 2100° to approximately 1300°; while for low carbon steels the solidification temperature ranges from 2550° F. to approximately 1650° F. Also, as is well known, for many steels the desired rolling temperature is very high, for example, soft steel at about 2200° F. and spring steel at about 2000° F.

Our present invention may be carried out in any suitable mold. In carrying out the invention we prefer to use a metallic big-end-down mold, and to pour molten metal into the chamber to a suitable level below the top of the mold at a preferably, but not necessarily so, rate sufficient to produce a relatively rapid rise of molten metal in the chamber whereby initial peripheral side wall cooling by the mold of the upper portion of the poured mass horizontally or radially opposite the metallic side walls of the chamber occurs relatively quickly after commencement of side wall cooling of the lower portion of the poured mass and whereby inward radial cooling of the poured

mass for its height in contact with the metallic side walls of the mold progresses at a substantially uniform radial rate for a period of time, and continuing the side cooling at a preferred rate to produce a skin of substantially uniform thickness so that the skin will tend to shrink to a plane parallel, or substantially parallel, to the chamber face of the mold side walls. To increase the length of time which the ingot skin would normally be in contact with the side walls of the mold and lengthen the time of relatively fast freezing and thereby thicken the skin or shell of the ingot by the formation of small crystals to a greater radial depth, the vertical mold body is moved in sliding contact with the ingot skin and during the sliding contact the side wall cooling is continued at a preferred rate to thicken the skin substantially uniformly inwardly for the length or height of the skin between the molten interior and the chamber walls. Preferably, the downward progression of the mold body is extremely slow, at least in its early stage, relative to the ingot skin shrinkage and its settling down in the mold, and, again preferably, the downward movement of the mold is under way while the shell of the ingot is relatively compressible or is sufficiently compressible to be laterally moved inwardly by the mold body so that the plane of the outer surface of the skin will be parallel for the major portion of its height with the inner face of the side walls of the mold. During at least some of the time the ingot shell is relatively compressible or movable inwardly by the mold body we prefer to remove or diminish the support for the mold body at a rate which will give support to the mold body during its downward progression to prevent a sudden drop. In some instances after the formation of a suitably thick skin or shell by slow sliding contact, and while the shell is relatively movable inwardly by the mold body and the interior is still molten, we prefer to withdraw the support from the mold body to cause the mold body to effect a relatively quick inward movement of the ingot shell so that the width of the container, so to speak, of the fluid portion is narrowed and the molten interior forced upwardly. Preferably, to improve the squeezing effect of the mold body on the ingot shell suitable force is employed to urge the mold body downwardly. After this squeezing action the mold body may, in desirable instances, be allowed to remain hanging on the skin of the ingot to continue its downward progression as contraction of the ingot or expansion of the mold permits. Any suitable mutable support may be used to support the mold body longitudinally movable relatively to the bottom-closure of the ingot-forming chamber, or any suitable combination of elements; we prefer to use a support susceptible to combustion, composed of any suitable element or combination of elements such as wood of any suitable degree of hardness or softness, in laminated assembly or otherwise, or in combination with another element or elements, or coke, or coal, or a mixture of sand and a combustible binder. The use of a combustible support to mutably support the mold body, as pointed out in our application for patent which is issuing as Patent No. 2,281,718, on May 5, 1942, supplies during burning heat in the lower portion of the mold and retards dissipation of heat generally from the lower portion of the ingot and mold, altering the cooling rate of the mold in the lower regions by slowing up the cooling rate, and preventing, or tending to prevent, the lower portion of the ingot from contracting

too fast relative to the lower portion of the mold walls and shrinking away therefrom while the upper portion of the ingot is in contact the walls of the mold during the relative body movement, and, in addition, the heat supplied by the combustion of the support assists in maintaining the lower portion of the ingot shell relatively movable or compressible in this region for at least a part of the time the side of the shell may be forced towards the axis of the mass. In the present invention we prefer to exercise control over the rate of combustion of the combustible support and vary its rate of combustion, preferably in the later stage of the downward progression of the mold body by increasing the rate of combustion to accelerate the burning, therefore the withdrawal, of the support of the mold body to effect a squeeze of the molten interior and at the same time increase the temperature of the heat supplied to the lower portion of the mold, and in some instances if desired, we may use a combustible support such as coke in any suitable form which is capable of evolving great heat, or such a combustible support in combination with any other suitable element or elements. When using a combustible support capable of evolving great heat and when varying the temperature of the heat, for example by increasing it for above cited purposes and or for the purpose of retarding the cooling of the lower portion of ingots intended to be charged hot into soaking pits or a reheating furnace, heat of relatively high temperature to the solidification temperature of the particular grade of steel or alloy of steel may be produced but low enough relatively thereto and relatively to the solidification temperature or temperatures of affected mold parts as not to cause fusion of the casting, or deformation or fusion of the mold.

In some instances in the present invention, especially in casting steel or alloys of steel subject to the formation of relatively deep cavities or pipe at the upper end of the ingot we may prefer after the formation preferably of a substantially uniform skin to the desired radial depth, to alter the side wall of radial cooling rate of the upper portion of the metallic mold walls by retarding the dissipation of heat therefrom while the interior of at least the upper portion of the ingot is still molten, and preferably by retarding the dissipation of heat at a progressively increasing rate upwardly, and thereby cool or solidify, as the case may be, the upper portion of the ingot horizontally opposite the metallic walls of the mold progressively upwardly. This we accomplish by teeming the molten mass into a mold having side walls of substantially uniform heat absorbing power or having side walls of relatively greater heat absorbing power opposite the wall contacting levels of molten mass last to rise than the cooling power of the walls relative to the cross-section of the poured mass at lower levels, having in mind the size and relative dimensions of the ingot-forming chamber, and preferably the pouring rate; and allowing solidification to progress for an interval of time at the rate of cooling predetermined by the fixed mass of the metallic side walls of the mold and the relationship of the mass of the vertical side walls to the ingot-forming chamber, and pouring the molten metal into the chamber at a temperature sufficiently high above the freezing point of the molten metal relative to the relationship of the cross-sectional thickness of the side walls of the mold to the cross-section of the ingot-forming chamber so that heat absorbed by the mold walls

from the poured mass will heat the outer metallic periphery of the upper portion of the mold while the interior of at least the upper portion of the poured mass is still molten radially opposite the upper portion of the inner metallic periphery of the ingot-forming chamber; and then, after the formation of the desired skin thickness, altering the predetermined cooling rate of the side walls of the mold by slowing up, progressively upwardly, the heat conductive rate of the upper portion of the side walls by retarding dissipation of absorbed heat from the surface of the outer periphery of the metallic mold body opposite the ingot contacting surface and "storing," so to speak, the absorbed heat in the walls to delay dissipation of heat from the solidifying ingot. This may be accomplished in any suitable manner and by any suitable means known in the art. We prefer to accomplish this by applying externally to the mold walls a conservator of heat surrounding the outer periphery of the vertical mold body and adapted to retard dissipation of heat from the upper portion of the mold, and which includes a circumferentially extending body of low heat conducting power encased in a durable frame, and a compressible elastic material of low heat conducting power, such as asbestos, to serve as a resiliently yieldable heat-insulating facing to peripherally engage, or substantially peripherally engage the outer surface of the vertical mold body.

In carrying out the invention with ingots of large section or generally large size, or in casting such or ingots of the various grades of steel, or in the casting of ingots generally, especially in big-end-down molds, it may be desirable in many instances to supply a relatively large volume of heat to the lower portion of the mold, particularly to the support for the ingot base, and in desirable instances, also, in which for reason of loss of heat in the mold by virtue of increased length of time of side wall contact of the mold with the ingot skin, the time required for a particular ingot to remain in the soaking pit or reheating furnace, that is an ingot charged hot therein, in preparation for rolling, may be reduced, relatively, by considerably retarding the loss of heat from its lower portion or bottom. By burning a combustible material capable of evolving great heat under the base support of the ingot, for example a combustible material such as coke, and regulating a supply of compressed air under suitable pressure, heat of relatively high temperature may be produced to considerably retard the dissipation of heat from the bottom and lower portion of the ingot at any desired stage; in casting steels of high solidification temperatures, this supplied heat of relatively high temperature will in most instances be considerably below, as a general practice, the temperature of solidification of the metal being cast, while in casting steels of low solidification temperatures, the temperature of supplied heat will be closer to the solidification temperature of the metal being cast.

Referring to the drawing:

Figure 1 is a vertical sectional view of an ingot mold assembly with parts of the apparatus shown in section and parts in elevation.

Figure 2 is a vertical sectional view of a modification of ingot mold assembly with parts of the apparatus shown in section and parts shown in elevation.

Figure 3 is a fragmentary vertical sectional

view of the ingot mold assembly shown in Fig. 2 equipped with a hot top.

Figure 4 is a fragmentary vertical sectional view of a modification of parts.

Referring to the drawing in more detail: In Fig. 1, on a suitable primary support 5, such as a floor, platform or transfer car, a generally rectangular metallic stool 6, preferably of cast iron, is supported on legs intermediate which the bottom of the stool is spaced from the primary support. Centrally in the stool a relatively large recess 7 is provided of generally rectangular shape with rounded corners and into which intermediate the corners laterally project a plurality of spaced tooth-like projections 8 which are integral parts of the metal of the stool and have their upper faces in the same plane and rigidly support a removable rectangular metallic plug-like bottom-closure 10 with rounded corners and which is preferably provided with a continuous laterally projecting ledge 9, integral therewith, and preferably of cast iron. The bottom-closure on its upper side is preferably provided with a relatively deep and wide recess surrounded by a rim of metal decreasing in cross-section towards the top. In the recess 7 below the plug-like bottom-closure is provided a suitable quantity of combustible material, preferably in the form of coke, as shown, in suitable sizes, which is capable of evolving great heat. Surrounding the plug-like bottom-closure is a continuous channel, rounded or curving at the corners, and in the channel is a mutable support 12 supporting a vertical mold body 13 which upon withdrawal or diminution of the mutable support will descend downwardly into the channel and downwardly relatively to the rigidly supported plug-like bottom-closure. The mutable support may be of any suitable material, and is preferably of combustible material, and may be of any suitable combustible material for example coal or coke in any suitable form or sizes, or any suitable wood or woods. In some instances the combustible support may consist of suitable lengths of wood accommodatable in the straight portions of the channel and at the rounded corners pieces of wood of small section may be stood on their ends and stacked in groups at the corners. Sealing material preferably of argillaceous material, such as fire clay, having the consistency of heavy tar is applied on the inner side of the upper face of the combustible support and the outer side of the upper end of the rim of the bottom-closure. Enough argillaceous material is provided so that the vertical mold body as it is positioned will squeeze it or bulge it so that it will extend from the rim of the plug to the inner periphery of the mold at the bottom and prevent the formation of a fin on the ingot. The vertical mold body is a big-end-down mold having the cross-sectional thickness of the wall moderately diminishing upwardly and is of rectangular shape with rounded corners externally and internally. The inner peripheral wall 14 of the body tapers, preferably moderately, inwardly in the upward direction, is preferably smooth, and may be coated, if desired, with any suitable material or wash known in the art. The height of the combustible support is such as to provide the desired amount of drop of mold relatively to the taper of the chamber, and relatively to the direction of increasing width of the chamber and the direction, or directions, or resultant direction of shrinkage or contraction of the ingot or expansion of the mold walls. In some instances we

prefer, without increase of mass of mold, to superimpose on the mold, preferably upon its outer peripheral side, a body of great weight which will act as a force to urge the mold body downwardly or at a desired stage will force the mold body downwardly, and in the early stages of the casting the body of great weight may be removably supported independently of the mold and later its weight caused to bear on the mold. As shown herein the outer peripheral side of the vertical mold body is provided with a plurality of laterally projecting tooth-like portions upon which is suspended a circumferentially continuous (ring-like) symmetrically balanced body of great weight 15 preferably provided with a facing 16 of heat-insulating material spaced from the peripheral side of the mold a suitable distance and which is wide enough in opposite portions to permit lowering of the body past lifting lugs commonly a part of ingot molds. In the stool below the combustible material 11 is a chamber 17 from which a vertical passage extends to the bottom of the stool and in the vertical passage is a forcibly fitted pipe having an externally threaded outer end projecting from the bottom of the stool. From the chamber extend a suitable number of suitably arranged passages 18 communicating with the recess in which the combustible material 11 is positioned to distribute air to the combustible material. Extending outwardly from the channel through the sides of the stool are a plurality of passages 19, preferably longitudinally and vertically spaced on the sides of the stool. Also communicating with the channel from the outer sides of the stool are a plurality of passages 20 shown in dotted lines, of suitable number and arrangement, in series. Provided in the stool, also, are two L-shaped passages 21 and 21a extending horizontally as elbowed pipes each having one longitudinal end closed and the other end communicating with the outer sides of the stool, preferably laterally of the corners, the latter ends being obliquely or diagonally opposite each other and being provided with forcibly fitted short pipes having their outer ends externally threaded and projecting outwardly from the sides of the stool. At suitably spaced distances from each other and laterally offset to the passages 20 are a series of 50 passages communicating with the channel from the L-shaped passages 21. Communicating with the recess 7, in locations laterally of the tooth-like projections 8 are a series of passages 22. In some instances we provide means to close or for practical purposes to temporarily close, from the atmosphere the outer ends of the passages 19, 20 and 22 by removable covers 23 suspended upon the stool, along each flat side thereof, and which can be easily removed at any desired period of the casting, and also, in some instances we may place argillaceous material between the bottom of the outer periphery of the mold and the stool wall at the outer side and upper end of the channel. The removable covers will serve principally to prevent, other factors being considered, such metal as may be tapped in a supermolten state from causing too early reduction of the combustible support relative to initial skin formation by the heat absorbing power of the mold. Connected to the externally threaded projecting ends of the pipe passages 21 and 21a respectively are internally threaded couplings on one end of flexible metal hose 24 and 25, the opposite ends of which are connected to a flexible metal hose 26 from which it may be closed or

to which it may be opened by a valve 28 from a pipe 30 connected to a supply pipe 5 communicating with a compressed air main A which is supplied with compressed air by an air compressor, not shown. Connected to the externally threaded projecting pipe end of the vertical passage communicating with the chamber 17 is an internally threaded coupling on the end of the flexible metal hose 27, the other end being connected to the pipe 30 from which it may be closed or to which it may be opened by the valve 29. The valve 28 provides control of the compressed air supply to the combustible support, and the valve 29 provides control of compressed air supply to the combustible material, coke as shown, in the recess 7, the valve 31 being normally open. In instances in which it may be desirable to jointly control the supply of compressed air to both the combustible support and combustible material the valve 31 will serve, valves 28 and 29 then being normally open; or in instances in which it may be desirable to jointly control the supply of compressed air to the combustible support and combustible material in a plurality of molds the valve 32 will serve, the others being open in that event. In assembling the mold parts the plug-like bottom-closure is positioned on the tooth-like supports 8 after the broken size coke is placed in the recess. The outer periphery of the plug provides the inner side wall of the channel which is preferably of uniform width. The ledge may in some instances co-operate with the stool to center the plug or the width of the mutable support in block form may do so, and when for any desirable reason the periphery of the plug, for insertion or removal purposes, is relatively widely spaced from the side of the recess such space may be filled with argillaceous material. The preferred pouring rate is such as will provide a relatively rapid rise of metal in the chamber whereby side wall cooling of the upper portion of the poured mass will occur relatively quickly after commencement of sidewall cooling, but this need not be so as heat may be supplied to the bottom of the mold to arrest the cooling of the lower portion of the poured mass at any desirable time after commencement of pouring, especially so in casting large ingots, particularly those long and wide and poured at usual or at slow rates to avoid splash or for other reasons. The construction shown in this figure of the vertical mold body is such that the thickness of mold wall decreases upwardly proportionally to the decrease upwardly of chamber section, and in some instances, particularly with long, wide chambers, the mold wall, may with advantage, decrease in thickness relatively less in relation to decrease of chamber section. The molten metal is poured to a height in the chamber which will provide a distance from the top of the mold to the top of the poured mass which is preferably greater than the distance which will be traversed by the downward progression of the mold body. Heat from the poured mass is conducted preferably by both the plug and mold body to the mutable support to burn it and combustion is supported by removing the covers 23 at the desired time. The origination of combustion may, if desired, be predetermined by the nature of the combustible support. Preferably the combustion of the support in the early stages is such as to provide a slow reduction and consequently a slow downward progression of the mold which progression begins after the formation of a suitable skin on

the poured mass, and it will be observed that the direction of mold movement relative to the base support of the ingot will tend not only not to elongate the skin relatively to the molten interior when the skin is movable inwardly by the mold but will force or tend to force the molten interior upwardly relatively to the skin, and further while the skin or any parts of the skin are relatively movable by the mold the direction of the mold movement relatively to the direction of longitudinal shrinkage of the skin is less apt to tear or crack the skin. Compressed air will be introduced to the combustible support principally for the purpose of rapidly burning the support and withdrawing it as a control of extent of drop of the mold at the desired stage to permit the body of great weight to force the mold body downwardly. Heat from the poured mass conducted by the plug will burn the combustible material, coke, and compressed air will be introduced to the chamber 17 and distributed to the coke to support combustion at the desired stage, the supply of air being controlled as desired and the temperature of the heat being increased, as desired under the circumstances of the particular casting.

In some instances steel or steels may be cast in metallic molds having greater cooling power of mold wall in the upper portion relatively to the cross-section of the upper portion of the chamber than the cooling power of the lower side walls relatively to the cross-section of the lower portion of the chamber, such a construction being shown in Fig. 2, wherein the thickness of the mold side walls 13a is uniform and the section of the chamber tapers moderately upwardly. Flexible metal hose 33 is connected to the passage 21a and flexible metal hose 34 is connected to the passage 21; the hose 33 and 34 being connected to flexible metal hose 35 connected to the pipe 39; flexible metal hose 36 is coupled to the threaded projecting pipe end in the vertical passage connecting with the chamber 17, the valves 37 and 38 corresponding to the valves 28 and 29, and the valve 40 corresponding to the valve 31. Surrounding the upper portion of the vertical mold body is a conservator of heat 41 durably constructed of a metallic frame or casing 42 housing a body of heat-insulating material of very low heat-conductivity, and on the inner peripheral face of the frame is preferably a facing of compressible elastic heat-insulating material, for example asbestos. The conservator is made of two parts bolted or riveted together and is provided on opposite sides with recess or pockets to accommodate the lifting lugs commonly a part of ingot molds, and is provided with upright supports 45, and is supported in spaced relation, preferably, to the outer periphery of the mold on removable blocks 46 which, in this instance rest on the body of great weight carried by the mold. The conservator of heat is a sleeve-like structure shaped to conform to the mold with its inner peripheral wall paralleling the plane of the outer periphery of the mold, and is longitudinally dropped and seated against the mold by removal of the blocks 46. After the formation of a suitably thick skin of substantially uniform thickness produced by sidewall cooling and when it is desired to alter the cooling of the upper portion of the poured mass, the conservator of heat will retard the dissipation of heat from the outer periphery of the mold and retard, progressively upwardly, the cooling or solidification of the molten interior of the ingot. In some instances

the mold may be equipped with a hot-top as shown in Fig. 3, hot tops being commonly used in the casting of deoxidized or killed steels to keep molten a supply of metal for feeding downwardly into the interior to bring the pipe to the upper end of the ingot. The refractory hot top 47 is supported by the top of the mold being provided with projections 48 to rest on the end of the mold. As the mold moves downwardly in sliding contact with the skin of the ingot the hot top is left upon the poured mass. In some instances in casting long ingots compressible elastic or combustible material may be interposed between the end of the mold wall and the projections 48.

In some instances after movement of sliding contact with the ingot skin of the vertical mold body stripping will be facilitated by lowering the ingot and the risk of skin damage such as tears avoided. In the modification of structure shown in Figure 4 the ledge 9 of the plug-like bottom-closure is provided with a suitable number of laterally projecting portions 9a to co-operate with the walls of the recess to serve to position and guide the plug, the upper end of the wall opposite the projections being rounded to facilitate seating the plug, the projections preferably extending into accommodating vertical shallow channels in the recess wall; the vertical channels extend to holes 49 in the lower part of the stool 6a. Having their lower portion in the holes in a sliding fit and the outer sides of their upper portions in the vertical shallow channels are a plurality of strong metal supports 50 provided with laterally projecting teeth 51 at their upper ends supporting the plug and are supported at their bottom ends by removable wedges 52 extending beneath the stool which at their thick ends are provided with obtusely projecting faces 53 on laterally projecting end portions 54 to facilitate their withdrawal by use of a sledge or other forcing tool. After sliding contact of mold with ingot skin and also the reduction of the coke, removal of the wedges will lower the plug and the ingot supported thereon spacing the ingot the desired distance from the side walls of the mold. As an additional modification and advantage the outer wall 55 of the channel will cooperate with the extreme marginal end of the mold body 13b which, while in other respects is the same as previously described, is in this instance provided with an outer periphery whose extreme marginal ends have a surface 56 paralleling and cooperable with the channel wall 55 to guide the mold body in its downward progression, the wall 57 in the stool being rounded to facilitate positioning the mold in the assembly.

The invention is susceptible to variations of forms, proportions and details within the broad principle without departure from the spirit of the invention, and having described it in its preferred form for purposes of illustration and not for limitation, we claim:

1. A method of casting ingots including pouring molten metal into a vertical metallic mold provided with an ingot-forming chamber of tapering cross-section the larger end of which is down, at a rate sufficient to produce a relatively rapid rise of molten metal in the chamber whereby initial peripheral sidewall cooling by the mold of the upper portion of the poured mass radially opposite the metallic side walls of the chamber occurs relatively quickly after commencement of sidewall cooling of the lower portion of the poured mass and whereby inward cooling of the poured mass for its height in contact with

the metallic side walls of the mold progresses at a substantially uniform radial rate, continuing the side wall cooling at a substantially uniform radial rate to form a skin of solidified metal on the poured mass to confine the molten interior, and providing sliding contact between the skin of the forming-ingot and the side walls of the mold by moving the vertical mold body longitudinally downwardly relatively to the forming-ingot and the base support of said forming-ingot.

2. A method of casting ingots including pouring molten metal into a vertical metallic mold provided with an ingot-forming chamber of tapering cross-section, the larger end of which is down, absorbing heat basally from the poured mass and absorbing heat by the side walls of the mold at a substantially uniform radial rate to form a skin of solidified metal to confine the molten interior, providing sliding contact between said skin and the side walls of the mold and laterally compressing the poured mass by moving the vertical mold body longitudinally downwardly relatively to the forming-ingot and the base support of said forming-ingot and in the direction in which the ingot skin is longitudinally shrinking and settling down in the mold.

3. A method of casting ingots including pouring molten metal into a vertical metallic mold provided with an ingot-forming chamber of tapering cross-section, the larger end of which is down, absorbing heat basally, and cooling the poured mass along the metallic side walls of the mold at a radial rate sufficient to produce a skin on the poured mass of substantially uniform thickness to confine the molten interior, providing sliding contact between the side walls of the mold and the skin of the forming-ingot by moving the vertical mold body longitudinally downwardly relatively to the forming-ingot and the base support of said forming-ingot, and retarding during at least part of the downward progression of said vertical mold body the cooling of the lower portion of the ingot by supplying heat generated outside the ingot-forming chamber to the lower portion of the metallic mold.

4. A method of casting ingots including pouring molten metal into a vertical metallic mold provided with an ingot-forming chamber of upwardly tapering cross-section, absorbing heat basally, and cooling the poured mass along the side walls of the mold at a radial rate sufficient to produce a skin on the poured mass of substantially uniform thickness to confine the molten interior, providing sliding contact between the side walls of the mold and the skin of the forming-ingot by producing a relative longitudinal body movement between the side walls of the mold on the one hand and the forming-ingot and its base support on the other hand, and retarding the cooling of the lower portion of the ingot by supplying heat of relatively high temperature and generated outside the ingot-forming chamber to the lower portion of the metallic bottom-closure of said ingot-forming chamber.

5. In a method of casting an ingot in an ingot mold assembly including the combination of a vertically extending mold body provided with an ingot-forming chamber of upwardly tapering cross-section and a separable metallic bottom-closure mutually supported for relative longitudinal body movement of each other by a combustible support adapted to supply heat to the lower portion of the mold, the steps of pour-

ing molten metal into the chamber, absorbing heat basally, and cooling the poured mass along the side walls of the mold at a radial rate sufficient to produce a skin on the poured mass of substantially uniform thickness to confine the molten interior, thickening the skin by providing sliding contact between the side walls of the mold and the ingot skin by burning the combustible support and producing a relative longitudinal body movement between said side walls of the mold on the one hand and the poured mass and chamber bottom-closure on the other hand while at least the upper portion of said poured mass is relatively compressible, and varying the rate of combustion of the combustible support to quicken its diminution and to increase the temperature of the heat supplied to the lower portion of the mold by the combustion of said support.

6. A method of casting an ingot in a vertical metallic mold provided with an ingot-forming chamber of tapering cross-section, the larger end of which is down, which includes pouring molten metal into the chamber at a temperature sufficiently high above the freezing point of the molten metal relative to the relationship of the cross-sectional thickness of the side walls of the mold to the cross-section of the ingot-forming chamber so that heat absorbed by the mold walls from the poured mass will heat the outer metallic periphery of the upper portion of the mold and will heat up said mold walls throughout their cross-section in said upper portion thereof sufficiently to have partially solidified the poured mass and to have greatly retarded the heat absorbing rate of said mold walls in said upper portion thereof while the interior of at least the upper portion of the poured mass is still molten radially opposite the upper portion of the inner metallic periphery of the ingot-forming chamber, providing sliding contact between the skin of the partially solidified mass and the side walls of the mold by moving the side walls of the mold longitudinally downwardly relatively to the poured mass and the base support of said poured mass, and retarding the solidification of the upper portion of the poured mass radially opposite the upper portion of the metallic side walls of the chamber by circumferentially retarding the dissipation of heat from the outer peripheral metallic surface of the side walls of the mold in the upper portion radially opposite the ingot-forming chamber by closely surrounding said upper peripheral metallic surface with a body of heat-insulating material separable of said mold.

7. A method of casting an ingot in a vertical metallic mold provided with an ingot-forming chamber of tapering cross-section, the larger end of which is down, which includes pouring molten metal into the chamber at a rate to produce a relatively rapid rise of molten metal in the chamber whereby initial peripheral sidewall cooling by the mold of the upper portion of the poured mass radially opposite the metallic side walls of the chamber occurs relatively quickly after commencement of side wall cooling of the lower portion of the poured mass and inward radial cooling of the poured mass for its height in contact with the metallic side walls of the mold progresses at a substantially uniform radial rate for a period of time, and pouring said molten metal at a temperature sufficiently high above its freezing point relative to the relationship of the cross-sectional thickness of the side walls of the mold to the cross-section of the in-

got-forming chamber so that heat absorbed by the mold walls from the poured mass will heat the outer metallic periphery of the upper portion of the mold and will heat up said mold walls throughout their cross-section in said upper portion thereof sufficiently to have partially solidified the poured mass and to have greatly retarded the heat absorbing rate of said mold walls in said upper portion thereof while the interior of at least the upper portion of the poured mass is still molten radially opposite the upper portion of the inner metallic periphery of the ingot-forming chamber, providing sliding contact between the skin of the partially solidified mass and the side walls of the mold by moving the side walls of the mold longitudinally downwardly relatively to the poured mass and the base support of said poured mass, and retarding the solidification of the upper portion of the poured mass radially opposite the upper portion of the metallic side walls of the chamber by circumferentially retarding the dissipation of heat from the outer peripheral metallic surface of the side walls of the mold in the upper portion radially opposite the ingot-forming chamber by closely surrounding said upper peripheral metallic surface with a body of heat-insulating material separable of said mold.

8. A method of casting an ingot in a vertical metallic mold provided with an ingot-forming chamber of tapering cross-section, the larger end of which is down, and side walls having the same, or approximately the same, heat absorbing rate horizontally opposite the upper and smaller portion of said chamber as the heat absorbing rate horizontally opposite the lower and larger portion of said chamber, which includes pouring molten metal into the chamber at a temperature sufficiently high above the freezing point of the molten metal relative to the relationship of the cross-sectional thickness of the side walls of the mold to the cross-section of the ingot-forming chamber so that heat absorbed by the mold walls from the poured mass will heat the outer metallic periphery of the upper portion of the mold and will heat up said mold walls throughout their cross-section in said upper portion thereof sufficiently to have partially solidified the poured mass and to have greatly retarded the heat absorbing rate of said mold walls in said upper portion thereof while the interior of at least the upper portion of the poured mass is still molten radially opposite the upper portion of the inner metallic periphery of the ingot-forming chamber, providing sliding contact between the skin of the partially solidified mass and the side walls of the mold by moving the side walls of the mold longitudinally downwardly relatively to the poured mass and the base support of said poured mass, and progressively retarding upwardly the solidification of the upper portion of the poured mass radially opposite the upper portion of the metallic side walls of the chamber by circumferentially retarding the dissipation of heat from the outer peripheral metallic surface of the side walls of the mold in the upper portion radially opposite the ingot-forming chamber.

9. A method of casting an ingot in a vertical metallic mold provided with an ingot-forming chamber of tapering cross-section, the larger end of which is down, which includes pouring molten metal into the chamber at a rate to produce a relatively rapid rise of molten metal in the chamber whereby initial peripheral sidewall cooling

by the mold of the upper portion of the poured mass radially opposite the metallic sidewalls of the chamber occurs relatively quickly after commencement of side wall cooling of the lower portion of the poured mass and inward radial cooling of the poured mass for its height in contact with the metallic sidewalls of the mold progresses at a substantially uniform radial rate for a period of time, and pouring said molten metal at a temperature sufficiently high above its freezing point relative to the relationship of the cross-sectional thickness of the sidewalls of the mold to the cross-section of the ingot-forming chamber so that heat absorbed by the mold walls from the poured mass will heat the outer metallic periphery of the upper portion of the mold and will heat up said mold walls throughout their cross-section in said upper portion sufficiently to have partially solidified the poured mass and to have greatly retarded the heat absorbing rate of said mold walls in said upper portion thereof while the interior of at least the upper portion of the poured mass is still molten radially opposite the upper portion of the inner metallic periphery of the ingot-forming chamber, providing sliding contact between the skin of the partially solidified mass and the side walls of the mold by moving the sidewalls of the mold longitudinally downwardly relatively to the poured mass and the base support of said poured mass at least while the poured mass is relatively compressible and at least the upper portion of its interior is still molten, retarding during at least part of the downward progression of the mold walls the cooling of the lower portion of the poured mass by supplying heat generated outside the ingot-forming chamber to the lower portion of the mold, and progressively retarding upwardly the solidification of the upper portion of the poured mass radially opposite the upper portion of the metallic sidewalls of the chamber by circumferentially retarding the dissipation of heat from the outer peripheral metallic surface of the side walls of the mold in the upper portion radially opposite the ingot-forming chamber.

10. A method of casting ingots including pouring molten metal into a vertical metallic mold provided with an ingot-forming chamber of upwardly tapering cross-section, absorbing heat basally, and cooling the poured mass along the side walls of the mold at a radial rate sufficient to produce a skin on the poured mass of substantially uniform thickness to confine the molten interior, providing sliding contact between the side walls of the mold and the skin of the forming-ingot by moving the side walls of the mold longitudinally downwardly relatively to the poured mass and the base support of said poured mass, and progressively retarding upwardly the solidification of the upper portion of the poured mass radially opposite the upper portion of the metallic side walls of the chamber by circumferentially retarding the dissipation of heat from the outer peripheral metallic surface of the side walls of the mold in the upper portion radially opposite the ingot-forming chamber while retarding the cooling of the lower portion of the ingot by supplying heat of relatively high temperature and generated outside the ingot-forming chamber to the lower portion of the metallic mold and to the bottom of the metallic bottom-closure of said ingot-forming chamber.

11. A method of casting ingots including pouring molten metal into a vertical metallic mold provided with an ingot-forming chamber of ta-

pering cross-section, the larger end of which is down, absorbing heat basally, and cooling the poured mass along the sidewalls of the mold at a radial rate sufficient to produce a skin on the poured mass of substantially uniform thickness to confine the molten interior, thickening the skin by providing sliding contact between the sidewalls of the mold and the ingot skin by moving the sidewalls of the mold longitudinally downwardly relatively to the ingot and the ingot base support, and later partially stripping the ingot by moving the ingot longitudinally downwardly relatively to the side walls of the mold.

12. An ingot mold assembly including the combination of a vertically extending metallic mold body provided with an ingot-forming chamber of tapering cross-section, the larger end of which is down, a separable metallic bottom-closure at said larger end of the ingot-forming chamber, and a mutable support disposed beneath said vertically extending mold body and supporting said mold body for downward longitudinal movement relatively to said bottom-closure.

13. An ingot mold assembly including the combination of a vertically extending metallic mold body provided with an ingot-forming chamber of tapering cross-section, the larger end of which is down, a separable metallic bottom-closure, a mutable support supporting the vertical mold body longitudinally movable relatively to said bottom-closure, and a removable body of relatively great weight superimposed upon the outer peripheral side of the vertical mold body.

14. An ingot mold assembly including the combination of a vertically extending metallic mold body provided with an ingot-forming chamber of tapering cross-section the larger end of which is down, and a metallic stool carrying a metallic bottom-closure for the chamber, said mold body being mutably supported for downward longitudinal movement relatively to the chamber bottom-closure, combustible material capable of evolving great heat provided in the stool and adapted to supply heat to the bottom of the bottom-closure, and means to force air to the combustible material.

15. An ingot mold assembly including the combination of a vertically extending metallic mold body provided with an ingot-forming chamber of tapering cross-section, the larger end of which is down, said mold body being mutably supported for downward longitudinal movement relatively to a metallic chamber bottom-closure carried by a stool, combustible material capable of evolving great heat provided in the stool and adapted to supply heat to the bottom of the bottom-closure, means to convey air to said combustible material to support combustion, and a removable body of relatively great weight superimposed upon the outer peripheral side of the vertical mold body.

16. An ingot mold assembly including the combination of a vertically extending metallic mold body provided with an ingot-forming chamber of tapering cross-section, the larger end of which is down, a separable metallic bottom-closure at said larger end of the ingot-forming chamber, a mutable support disposed beneath said vertically extending mold body and supporting said mold body for downward longitudinal movement relatively to said bottom-closure, and a removable body of relatively great weight superimposed upon the outer peripheral side of said mold body and having the weight of its mass substantially the same on, and substantially symmetrically dis-

tributed on, diametrically opposite sides of said mold body.

17. In casting apparatus, an ingot mold assembly including the combination of a vertically extending metallic mold body provided with an ingot-forming chamber of tapering cross-section, the larger end of which is down, a separable metallic bottom-closure, a combustible support mutably supporting the vertical mold body for downward longitudinal movement relatively to said bottom-closure and adapted to supply heat to the lower portion of the mold during diminution of said combustible support, rigid means in the assembly to support the combustible support, means to supply air to the combustible support, and means to control the supply of air to said combustible support for varying its rate of combustion.

18. Ingot casting apparatus including the combination of a vertically extending metallic mold body provided with an ingot-forming chamber of tapering cross-section, the larger end of which is down, a metallic stool provided with a rigidly supported plug-like bottom-closure at the larger end of the chamber, a continuous channel in the stool surrounding the bottom-closure and adapted to receive the lower marginal end wall of said vertical mold body, a combustible support in the channel mutably supporting the vertical mold body longitudinally movable downwardly relatively to the plug-like bottom-closure and adapted to supply heat to the bottom of said vertical mold body during diminution of said combustible support, rigid means in the stool to support the combustible support, a recess in said stool immediately below the bottom-closure, combustible material provided in said recess and adapted during combustion to supply heat to the bottom of said bottom-closure, means to convey a supporter of combustion to said combustible support, means to vary the rate of combustion of said combustible support, means to convey a supporter of combustion to said combustible material, and means to control and vary the rate of combustion of said combustible material.

19. Ingot casting apparatus including the combination of a vertically extending metallic mold body provided with an ingot-forming chamber of tapering cross-section, the larger end of which is down, a metallic stool provided with a rigidly supported plug-like bottom-closure at the larger end of the chamber, a continuous channel in the stool surrounding the bottom-closure and adapted to receive the lower marginal end wall of said vertical mold body, a combustible support in said channel mutably supporting said vertical mold body longitudinally movable downwardly relatively to said plug-like bottom-closure and adapted to supply heat to the bottom of said vertical mold body during diminution of said combustible support, rigid means in the stool to support said combustible support, a recess in said stool immediately below said bottom-closure, combustible material provided in said recess and adapted during combustion to supply heat to the bottom of said bottom-closure, means to convey a supporter of combustion to said combustible support, means for varying the rate of combustion of said combustible support, means to convey a supporter of combustion to said combustible material, means for controlling and varying the rate of combustion of said combustible material, and a removable body of relatively great weight superimposed upon said vertical mold body.

20. An ingot mold assembly including the com-

bination of a vertically extending metallic mold body provided with an ingot-forming chamber of tapering cross-section, the larger end of which is down, a separable metallic chamber-bottom-closure, means mutably supporting the vertical mold body for downward longitudinal movement relatively to said chamber-bottom-closure, and a sleeve-like conservator of heat adjustably supported relatively to and surrounding the upper portion of the outer periphery of the vertical mold body and including a relatively soft, elastic compressible elastic facing of heat-insulating material on its inner peripheral wall.

21. In casting apparatus, an ingot mold assembly including the combination of a vertically extending metallic mold body provided with an ingot-forming chamber of tapering cross-section, the larger end of which is down, and a separable metallic bottom-closure, a combustible support mutably supporting the vertical mold body for downward longitudinal movement relatively to said bottom-closure and adapted to supply heat to the lower portion of the mold during diminution of said combustible support, rigid means in the assembly to support the combustible support, means to supply air to the combustible support, means to control the supply of air to said combustible support for varying its rate of combustion, and a sleeve-like conservator of heat adjustably supported relatively to and surrounding the upper portion of the outer periphery of the vertical mold body and including a compressible elastic facing of heat-insulating material on its inner peripheral wall.

22. In casting apparatus, an ingot mold assembly including the combination of a vertically extending metallic mold body provided with an ingot-forming chamber of tapering cross-section, the larger end of which is down, and a separable metallic bottom-closure, a combustible support mutably supporting said vertical mold body for downward longitudinal movement relatively to said bottom-closure and adapted to supply heat to the lower portion of the mold during diminution of said combustible support, rigid means in the assembly to support said combustible support, means to supply air to said combustible support, means to control the supply of air to said combustible support for varying its rate of combustion, a removable body of great weight superimposed upon said vertical mold body, and a sleeve-like conservator of heat adjustably supported relatively to and surrounding the upper portion of the outer periphery of said vertical mold body and including a compressible elastic facing of heat-insulating material on its inner peripheral wall.

23. In ingot casting apparatus, an ingot mold assembly including the combination of a vertically extending metallic mold body provided with an ingot-forming chamber of tapering cross-section, the larger end of which is down, a metallic stool provided with a rigidly supported plug-like bottom-closure at the larger end of the chamber, a continuous channel in the stool surrounding the bottom-closure and adapted to receive the lower marginal end wall of said vertical mold body, a mutable support in the channel supporting the vertical mold body for downward longitudinal movement relatively to the plug-like bottom-closure, and means on the outer peripheral side of the vertical mold body at the bottom marginal end thereof co-operable with means on the outer side wall of the channel in the stool for guiding the downward movement of

the vertical mold body to prevent, or to substantially prevent, axial tilting of said vertical mold body.

24. An ingot mold assembly including the combination of a vertically extending metallic mold body provided with an ingot-forming chamber of upwardly tapering cross-section, a separable metallic chamber-bottom-closure, mutable means supporting said mold body for downward longitudinal movement relatively to said chamber-bottom-closure, and means independent of said mutable means supporting said chamber-bottom-closure for downward longitudinal movement relatively to said mold body.

25. An ingot mold assembly including the combination of a vertically extending metallic mold body provided with an ingot-forming chamber of tapering cross-section, the larger end of which is down, a metallic stool provided with a plug-like bottom-closure at the larger end of the chamber, a continuous channel in the stool surrounding the bottom-closure and adapted to receive the lower marginal end wall of said vertical mold body, a mutable support in the channel mutably supporting the vertical mold body longitudinally movable downwardly relatively to the plug-like bottom-closure, and movable rigid means supporting said plug-like bottom closure for downward longitudinal movement relatively to the vertical mold body.

26. Casting apparatus including in combination, a vertically extending metallic mold body provided with an ingot-forming chamber of tapering cross-section, the larger end of which is down, a metallic stool provided with a plug-like bottom-closure at the larger end of the chamber, a continuous channel in the stool surrounding the bottom-closure and adapted to receive the lower marginal end wall of said vertical mold body, a combustible support in the channel mutably supporting the vertical mold body for downward longitudinal movement relatively to the plug-like bottom-closure, means on the outer peripheral side of the vertical mold body at the bottom marginal end thereof cooperable with means on the outer side wall of the channel in the stool for guiding the downward movement of the vertical mold body to prevent, or substantially prevent, axial tilting of said vertical mold body, movable rigid means supporting the plug-like bottom-closure for downward longitudinal movement relatively to the vertical mold body, a recess in the stool immediately below the bottom-closure, combustible material capable of evolving great heat provided in said recess and adapted during combustion to supply heat to the bottom of said bottom-closure,

sure, means to supply air to the combustible support, means to supply air to said combustible material, means to control the supply of air to said combustible support and said combustible material for varying their rates of combustion, and a sleeve-like conservator of heat adjustably supported relatively to and surrounding the upper portion of the outer periphery of the vertical mold body and including a compressible elastic facing of heat-insulating material on its inner peripheral wall.

27. Casting apparatus including in combination, a vertically extending metallic mold body provided with an ingot-forming chamber of tapering cross-section, the larger end of which is down, a metallic stool provided with a plug-like bottom-closure at the larger end of the chamber, a continuous channel in the stool surrounding said bottom-closure and adapted to receive the lower marginal end wall of said vertical mold body, a combustible support in said channel mutably supporting said vertical mold body for downward longitudinal movement relatively to said plug-like bottom-closure, means on the outer peripheral side of said vertically extending mold body at the bottom marginal end thereof cooperable with means on the outer side wall of said channel in said stool for guiding downward movement of said mold body to prevent, or substantially prevent, axial tilting of said mold body, a removable body of relatively great weight superimposed upon the outer peripheral side of said mold body and having the weight of its mass the same on, and symmetrically distributed on, diametrically opposite sides of said mold body, movable rigid means supporting said plug-like bottom-closure for downward longitudinal movement relatively to said mold body, a recess in said stool immediately below said bottom-closure, combustible material capable of evolving great heat provided in said recess and adapted during combustion to supply heat to the bottom of said bottom-closure, means to supply air to said combustible support, means to supply air to said combustible material, means to control the supply of air to said combustible support and to said combustible material for varying their rates of combustion, and a sleeve-like conservator of heat adjustably supported relatively to and surrounding the upper portion of the outer periphery of said vertically extending mold body and including a compressible elastic facing of heat-insulating material on its inner peripheral wall.

55

JOHN T. SCULLY.  
GEORGE H. WYCKOFF.